# EUROPEAN PATENT SPECIFICATION

(11) **EP 0 111 564 B1**
(45) Date of publication and mention of the grant of the patent: **09.09.1987**
(21) Application number: 83901395.0
(22) Date of filing: 04.05.1983
(51) Int. Cl.: B41M 5/22

(54) **COLOR-DEVELOPING SHEET FOR PRESSURE-SENSITIVE RECORDING**
FARBENTWICKLERBLATT FÜR DRUCKEMPFINDLICHE AUFZEICHNUNG
FEUILLE DE DEVELOPPEMENT COULEUR POUR ENREGISTREMENT SENSIBLE A LA PRESSION

(30) Priority: 22.06.1982 JP 107022/82
(43) Date of publication of application: 27.06.1984
(73) Proprietor: MITSUBISHI PAPER MILLS, LTD., Chiyoda-ku Tokyo 100 (JP)
(72) Inventor: TORII, Takahiro, Kako-gun Hyogo 673-01 (JP); SENOH, Hideaki, Takasago-shi Hyogo 676 (JP); TSUKAHARA, Hirokazu, Takasago-shi Hyogo 676 (JP)
(74) Representative: Hansen, Bernd, Dr. Dipl.-Chem.
(86) International application number: JP8300137
(87) International publication number: WO8400131

## Description

This invention relates to a color-developing sheet having a novel constitution for pressure-sensitive recording.

The pressure-sensitive recording material comprises usually a color-forming sheet having an electron-donative leuco dye on the surface and a color-developing sheet having a color developer, which is electron attractive, on the surface. In this recording material, a color-forming reaction based on electron transfer is utilized for recording by bringing both the surfaces into contact with each other and applying printing pressure thereto.

Accordingly, the color developer is one of the principal components of this recording material and various color developers have hitherto been proposed. For example, there have been proposed activated clay, which is obtained by treating a natural clay mineral with acid to a slight or medium extent, phenol compounds, phenolic resins of novolak type, and metal salts of aromatic carboxylic acids.

Activated clay first mentioned, which is the oldest of the above color developers, is insufficient in an essential property, i.e. the color developing ability. Hence, there are cases where activated clay has been replaced with some of the above-mentioned organic color developers.

On the other hand, a novel color developer has been proposed recently which is prepared by a semi-synthetic process (EP-A-44 645).

It is a color developer for use in pressure-sensitive recording materials which is prepared in the following way: A clay mineral having a layer structure build up of regular tetrahedrons of silica is treated with an acid so as to give a silica content of 82-96.5% by weight on a dry basis (dried at 105°C for 3 hours); a magnesium component and/or aluminum component is introduced into the acid-treated clay mineral by bringing it, in an aqueous medium, into contact with a magnesium compound and/or aluminum compound soluble at least partially in the medium and if this soluble compound is other than the hydroxide, by neutralizing it with alkali or acid to form the hydroxide; and if desired, the resulting clay mineral is dried (hereinafter this color developer is referred to as "semi-synthetic solid acid"). The clay mineral resulting from the above process shows the following characteristics: (a) an electron diffraction pattern based on the crystals of the above layer structure built up of regular tetrahedrons of silica, (b) no X-ray diffraction pattern based on the above layer structure, and (c) contains at least silicon and magnesium and/or aluminum as elements besides oxygen. This new clay mineral has brought about an improvement in the color-developing ability for electron-donative leuco dyes, long lasting of the color-developing effect under high humidity conditions, and less decay with time of the formed color density. Thus, the semi-synthetic solid acid can be regarded as a new type of color developer capable of offsetting sufficiently drawbacks of conventional activated clays and expected to be comparable or superior in the color developing ability to organic color developers.

The present inventors evaluated by various tests the aptitude of the semi-synthetic solid acid, which is a new type of inorganic color developer prepared in the above process, for use in the color-developing layer for pressure-sensitive recording. As a result, a marked improvement in the color developing ability and a good retention of the colored image density under high humidity conditions were surely recognized and hence distinct differences were observed between this semi-synthetic solid acid and the clay mineral group color developer so far known and used. On the other hand, it was found as a drawback of the semi-synthetic solid acid that some fastness, for example, light fastness, of the color image formed in the color-developing layer employing the semi-synthetic solid acid is rather deteriorated.

In view of the above, the present inventors made extensive studies in the search for a means of improving the fastness of the color image formed in such a color-developing layer. As a result, this invention has been accomplished through new finding that the addition of any of various known antioxidants such as aromatic amines and hindered phenols and any of ultraviolet absorbers such as benzotriazole derivatives is little effective, but the addition of necessary amounts of a phenol compound and a zinc-compound markedly improves the light fastness of the color image formed; in particular the use of a selected phenol compound together with a zinc compound gives a semi-synthetic solid acid-containing color-devloping layer really excellent in practical use which does not cause any objectionable side reaction such as the yellowing of the blank areas (image-less areas on the color-developing layer).

Thus, the invention comprises:
a color-developing sheet for pressure-sensitive recording, wherein the color-developing layer of the sheet contains
   (A) a color-developer for pressure-sensitive recording paper which is derived by acid treatment from a clay mineral having a layer-structure composed of regular tetrahedrons of silica and which shows
      (a) a diffraction pattern attributable to crystals of layer-structure composed of regular tetrahedrons of silica when subjected to electron diffraction analysis, but
      (b) no diffraction pattern attributable to the crystals of said layer-structure when subjected to X-ray diffraction analysis, and
      (c) contains as constituent elements besides oxygen, silicon and magnesium and/or aluminum, and is

      characterized in that it contains further
      (B) a phenol compound and
      (C) a zinc compound.

The phenol compound used jointly with the semi-synthetic solid acid in this invention may be either a low molecular weight phenol compound or a phenolic resin. Especially suitable phenol compounds which do not cause such a side reaction as the discoloration or coloration of the blank areas or the degradation are, for example, alkyl, aralkyl or aryl p-hydroxybenzoates, (like those disclosed in EP-A-105 376 which constitutes prior art according to Article 54(3) and (4) EPC).

p-hydroxybenzonitrile, p-hydroxybenzenesulfonamide, 4-hydroxybenzophenone, 2,4-dihydroxybenzophenone, dialkyl, diaralkyl, or diaryl 4-hydroxyphthalic acid esters, and various hindered phenols. Suitable amounts thereof used are 1-100 parts per 100 parts of the semi-synthetic solid acid.

Especially effective zinc compounds used in this invention are, for example, zinc oxide, zinc hydroxide, zinc carbonate, basic zinc carbonate, zinc sulfide, zinc phosphate, and zinc salts of various organic acids. Suitable amounts thereof used are 1-100 parts per 100 parts of the semi-synthetic solid acid.

Preferred examples of the color developer for pressure-sensitive copying paper used in this invention satisfy the above conditions (a), (b), and (c) and additionally the condition that (d) the atomic ratio of [silicon]/[the sum of magnesium and/or aluminum] therein is 12/1.5-12/12, particularly 12/3-12/10. Herein, when only one of magnesium and aluminum is contained, the sum of magnesium and/or aluminum in the above atomic ratio means the amount of the contained one.

As stated above, it has been found in this invention that the combined use of the semi-synthetic solid acid, phenol compound, and zinc compound gives a color-developing sheet for pressure-sensitive recording materials which is far more improved in the fastness of the color image than does the use of the semi-synthetic solid acid alone. Moreover, as will be shown later in Examples, the simultaneous addition of the phenol compound and zinc compound has excellent effects particularly in improving the fastness of the color image formed as compared with the separate addition of the compounds. That is, a synergistic effect is observed in the former case.

In this invention, the color-developing layer for pressure-sensitive recording is formed by; mixing the semi-synthetic solid acid, one or more of the zinc compounds, one or more of the phenol compounds, a binder, a dispersant, some other additive, and if desired, a pigment such as clay, kaolin, satin white, calcium carbonate, titanium white, magnesium oxide, talc, alumina, aluminum hydroxide, urea resin pigment, or plastic pigment, applying the resulting coating liquid on a sheet-like support such as paper, plastic film, plastic-coated paper, or the like by using an air knife coater, blade coater, roll coater, flexo coater, gravure coater, rubber doctor coater, curtain coater, or some other coating means; and drying the coat.

As described above, the color developing layer in this invention is formed by using the semi-synthetic solid acid as color developer and using cojointly the zinc compound and the phenol compound. In this way, this invention has been successful in providing a pressure-sensitive recording system unprecedentedly markedly improved in all the color forming rate, formed color density, fastness of the formed color image (to light, water, humidity, plasticizer, oxidizing gas, etc.), and stability (retention of color developing ability, resistance to yellowing) of the image-less areas (blank areas). In particular, it is noteworthy that the formed color density, the retention thereof under high humidity conditions, and the fastness of the formed color image to NOx are improved, the fading with light is reduced, and the blank areas do not undergo the yellowing.

Referring now to a typical example, preferred embodiments of this invention are illustrated in more detail. In the following example, "parts" are all by weight.

### Example

The following mixture was ball-milled for two days.

Then, 100 parts of a semi-synthetic solid acid (tradename: Silton SS-1, Mizusawa Chem. Ind. Co., Ltd.), 10 parts of zinc oxide, and 50 parts of the above dispersion of benzyl p-hydroxybenzoate prepared by the wet grinding were dispersed in 200 parts of water dissolving 1 part of sodium pyrophosphate. To the resulting dispersion were added 50 parts of a 10% aqueous solution of oxidized starch and 50 parts of a 48% SBR latex to prepare a coating liquid. It was coated on 40-g/m² base paper to give a dry coating weight of 4.5 g/m². Thus, color-developing sheets (CF) were prepared (sample D).

For the purpose of comparative tests, samples were prepared without adding either benzyl p-hydroxybenzoate or zinc oxide (sample A), without adding benzyl p-hydroxybenzoate but with adding the same amount of zinc oxide (sample C), and without adding zinc oxide but with adding the same amount of benzyl p-hydroxybenzoate (sample B) were prepared in the same manner as the above.

Color-forming sheets (CB) herein used were prepared as follows: A solution of electron-donative leuco dyes in a high boiling solvent having the composition:

was micro-capsuled with a melamine resin according to the method of US―A―4 233 178. To 100 parts (dry basis) of the micro-capsules were added 25 parts of wheat starch and 150 parts of a 10% aqueous solution of oxidized starch. The resulting mixture was coated on 40-g/m^{z} base paper to give a dry coating weight of 5 g_{/m2.}

A specimen of each of the thus obtained CF sheets (4 types) and a specimen of the CB sheets were superposed so as to oppose the coating surfaces and were super-calendered. After one or more days, tests of exposure to sunlight and room scattered light and other fastness tests were conducted on the thus colored specimens of the color-developing sheets (Table 1).

From Table 1, a synergy is observed in the effect of this invention. In other words, when (the retentions of the samples B, C, and D) (%)-(the retention of the sample A) (%) are designated as ΔB, ΔC, and ΔD(%) in the sunlight exposure tests, AB=11(%), AC=2(%), and ΔD=23(%) and therefore ΔD>ΔB+ΔC.

The same relations are found in the NOx exposure, room scattered light exposure, and plasticizer exposure test results.

Thus, according to this invention, much greater improvements in the fastness of the color image have been attained by combined use of the phenol compound and the zinc compound than by separate use of these compounds.

## Claims

1. A color-developing sheet for pressure-sensitive recording, wherein the color-developing layer of the sheet contains:
(A) a color-developer for pressure-sensitive recording paper which is derived by acid treatment from a clay mineral having a layer-structure composed of regular tetrahedrons of silica and which shows
(a) a diffraction pattern attributable to crystals of layer-structure composed of regular tetrahedrons of silica when subjected to electron diffraction analysis, but
(b) no diffraction pattern attributable to the crystals of said layer-structure when subjected to X-ray diffraction analysis, and
(c) contains as constituent elements besides oxygen, silicon and magnesium and/or aluminum,
characterized in that said layer contains further
(B) a phenol compound and
(C) a zinc compound.

2. A color-developing sheet for pressure-sensitive recording according to claim 1, characterized in that additional to the conditions (a), (b) and (c) the condition (d) is fulfilled according to which the atomic ratio of [silicon]/[the sum of magnesium and/or aluminum] is 12/1.5-12/12, particularly 12/3-12/10.

## Patentansprüche

1. Farbentwicklungsblatt für druckempfindliche Aufzeichnungen, wobei die farbentwickelnde Schicht des Blattes enthält:
(A) einen Farbentwickler für druckempfindliches Aufzeichnungspapier, der durch Säurebehandlung eines Tonminerals mit Schichtstruktur, zusammengesetzt aus regelmässigen Tetraedern aus Siliciumdioxid, erhalten wurde und der
(a) ein Beugungsbild zeigt, das den Kristallen der Schichtstruktur, die sich aus regelmässigen Tetraedern aus Siliciumdioxid zusammensetzt, zuzuschreiben ist, wenn man eine Elektronenbeugungsanalyse vornimmt, wobei jedoch
(b) kein Beugungsbild, das den Kristallen der Schichtstruktur zuzuschreiben ist, vorliegt, wenn man eine Röntgenbeugungsanalyse vornimmt, und
(c) als Bestandteil Elemente neben Sauerstoff, Silicium und Magnesium und/oder Aluminium enthält,
dadurch gekennzeichnet, dass die Schicht weiterhin
(B) eine Phenolverbindung und
(C) eine Zinkverbindung enthält.

2. Farbentwicklungsblatt für eine druckempfindliche Aufzeichnung gemäss Anspruch 1, dadurch gekennzeichnet, dass zusätzlich zu den Bedingungen (a), (b) und (c) die Bedingung (d) erfüllt ist, gemäss welcher das Atomverhältnis von [Silicium]/[Summe aus Magnesium und/oder Aluminium] 12/1,5 bis 12/12, insbesondere 12/3 bis 12/10, beträgt.

## Revendications

1. Feuille de développement en couleur pour enregistrement par pression, dans laquelle la couche de développement de couleur de la feuille contient:
(A) un développateur de couleur pour papier d'enregistrement sensible à la pression, que l'on obtient, par traitement à l'acide, à partir d'un minéral argileux présentant une structure en couches, composée de tétraèdres réguliers de silice, et
a) qui présente un diagramme de diffraction attribuable à des cristaux de structure en couches composée de tétraèdres réguliers de silice, lorsqu'il est soumis à une analyse par diffraction des électrons,
b) qui, en revanche, ne présente pas de diagramme de diffraction attribuable aux cristaux de ladite structure en couches, lorsqu'il est soumis à une analyse par diffraction des rayons X, et
c) qui contient, en tant qu'éléments constitutifs, outre l'oxygène, du silicium et du magnésium et/ou de l'aluminium,
caractérisée. en ce que ladite couche contient en plus
(B) un composé phénol, et
(C) un composé du zinc.

2. Feuille de développement en couleur par enregistrement par pression, conforme à la revendication 1, caractérisée en ce que, en plus des conditions a), b) et c), est remplie la condition d) selon laquelle le rapport atomique [silicium]/[somme du magnésium et de l'aluminium] est compris entre 12/1,5 et 12/12, et en particulier entre 12/3 et 12/10.
